

## UNITED STATES PATENT OFFICE

ANDREW GUSTAVE KRANS, OF LOS ANGELES, CALIFORNIA, ASSIGNEE OF ONE-HALF TO  
JOHN S. KIRSTEIN, OF LOS ANGELES, CALIFORNIA

## ALLOY

No Drawing.

Application filed July 26, 1929. Serial No. 381,403.

This invention relates to alloys and, more particularly, those containing a relatively large percentage of copper.

An object of the invention is the production of an alloy having a greater tensile strength than steel, one that exactly matches the color of gold, and one that does not tarnish or oxidize to a sufficient extent to destroy its brightness.

10 This alloy is capable of use for the production of cutlery and jewelry.

Another object of the invention is to provide an alloy which can be made to closely imitate various gold tone colors by a variation 15 in the amount of one of the ingredients.

Other objects and advantages will appear in the subjoined detailed description.

The metals employed in the production of this alloy are copper, tin, nickel, aluminum 20 and beryllium. These metals are melted together by placing them in a heated crucible, and the temperature employed ranges from approximately 2300° F. to 2400° F.

After the alloy thus produced has cooled, 25 it will melt when raised to a temperature of approximately 1900° F.

The above mentioned metals are used in the alloy in the following proportionate amounts: nickel approximately 1%, tin approximately 1/2 to 1%, aluminum approximately 5%, beryllium from approximately 1/16 of 1% to 1%, and the balance copper. These amounts are by weight.

35 The copper produces the gold tone, the tin brightens, the nickel and aluminum increase the tensile strength to some degree, and the beryllium further increases the tensile strength of the alloy. The different gold colors are secured by varying the amount of 40 tin employed in the alloy, the less tin employed the deeper the tone and the more tin employed the whiter the tone. Thus by varying the amount of tin, all the different shades of gold may be produced from the 45 deep golden color, through the various tones of yellow to white.

I claim:

An alloy characterized in that it contains from approximately 1/2 to 1 percent tin, approximately 1 percent nickel, approximately

5 percent aluminum, from approximately 1/16th of 1 percent to 1 percent beryllium, and sufficient copper to complete 100 percent.

Signed at Los Angeles, California, this 20th day of July, 1929.

ANDREW GUSTAVE KRANS.

55

60

65

70

75

80

85

90

95

100